

**3,447,980**  
**CASTABLE EXPLOSIVE CONTAINING TNT AND**  
**A REACTION PRODUCT OF A DIISOCYANATE**  
**AND 1,4-BUTYLENEOXIDE POLYGLYCOL**

H. William Voigt, Jr., Stanhope, N.J., assignor to the  
 United States of America as represented by the Secretary  
 of the Army  
 No Drawing. Filed Jan. 20, 1967, Ser. No. 610,697  
 Int. Cl. C06b 9/04

U.S. Cl. 149—19

5 Claims

**ABSTRACT OF THE DISCLOSURE**

A polyurethane modified castable high explosive, such as TNT or Petrin Acrylate, whose solidified cast is essentially free of voids, cavities, or exuding oils.

This invention relates to a castable high explosive of the type based on 2,4,6-trinitrotoluene or some analogous melt medium such as pentaerythritol acrylate trinitrate.

As is well known, castable high explosives are not only required in the manufacture of large caliber shells but are also preferred in the manufacture of other type shells due to simplicity in handling, safety achieved in loading, and overall cost in manufacture.

In the past, characteristics such as exudation, cavitation, brittleness, and irreversible expansion were noted in the preparation of a castable high explosive such as 2,4,6-trinitrotoluene. In the case of exudation, the low melting oils usually appear when the cast is stored around 71° C. but may appear even at room temperature. This leads to cavitation and independent spinning of the cast when the shell is fired from a rifled barrel. Also, the physical nature of the cast is usually brittle, particularly at the low temperatures required of military use, and cracking occurs when the cast is cycled from differing zones of temperature. The latter condition ultimately affects the impact sensitivity of the cast. Further, the coefficient of thermal expansion of this type castable explosive is high and irreversible expansion of the cast occurs when heated. This facilitates the formation of voids which also adversely influences the impact sensitivity of the final cast.

The subject invention essentially eliminates the aforesaid disadvantages which are inherent in the manufacture of cast explosives by treating such explosives during manufacture with a mild, two-component, liquid polyurethane-producing system.

It is therefore an object of this invention to provide a polyurethane modified castable high explosive whose solidified cast is essentially free of voids, cavities, or exuding oils.

Another object is to provide an improved high explosive cast which, as a result of its composition, exhibits a higher degree of impact strength and a lesser degree of brittleness when compared to similar explosives of the art.

TABLE I

| Composition                                | Control               | A                               | B                               | C                               |
|--------------------------------------------|-----------------------|---------------------------------|---------------------------------|---------------------------------|
| Percent by weight:                         |                       |                                 |                                 |                                 |
| TNT                                        | 100.                  | 55.                             | 75.                             | 95.                             |
| Urethane prepolymer                        |                       | 22.                             | 12.2                            | 2.4.                            |
| Curing Agent                               |                       | 11.                             | 6.1                             | 1.2.                            |
| Compatibilizer                             |                       | 11.                             | 6.1                             | 1.2.                            |
| Vacuum Stability: 5 g., 40 hrs. at 120° C. | 0-2 mls.              | 0-2 mls.                        | 0-2 mls.                        | 0-2 mls.                        |
| Crystallinity on solidification            | Large crystals formed | Amorphous or micro-crystalline. | Amorphous or micro-crystalline. | Amorphous or micro-crystalline. |
| Color of Cast                              | Off White             | Light Yellow                    | Light Yellow                    | Light Yellow                    |
| Shrinkage (melt to solid), percent         | 10                    | 5.5                             | 7.0                             | 9.                              |
| Case Bonding to Container                  | Negligible            | Firm                            | Firm                            | Firm                            |
| Exudation: 8 days, 71° C.                  | 0.42                  | None                            | None                            | None                            |
| Melting Range, ° C.                        | 79-80                 | >100                            | >100                            | >100                            |
| Physical Characteristics                   | Brittle               | Non-Brittle                     | Non-Brittle                     | Non-Brittle                     |
| Hardness (ASTM-D676-55T) Shore D:          |                       |                                 |                                 |                                 |
| 80° C.                                     | 0 (liquid)            | 33.                             | 33.                             | 15.                             |
| 20° C.                                     | 45.                   | 55.                             | 55.                             | 55.                             |
| -40° C.                                    | 60.                   | 65.                             | 65.                             | 65.                             |

As may be seen from the above cited data, the explosive composition incorporating the polyurethane producing system is highly stable, free of cracks and evidence of exudation, and substantially less brittle than the explosive composition which served as a control. Further, the treated explosive is firmly bonded to the containers while the control is only negligibly bonded and, as heretofore stated, the latter actions leads to independent spinning of the cast when fired.

A castable high explosive which is equivalent to TNT in this composition is pentaerythritol acrylate trinitrate also known as petrin acrylate. The latter explosive also exhibits exudation prior to treatment due to the incorporation of low melting plasticizers. Further, the TNT or petrin acrylate in the composition may be replaced with up to 80 percent by weight of cyclotrimethylene trinitramine, also known as RDX, or cyclotetramethylene tetranitramine which is conventionally known as HMX. Such replacement will tend to upgrade the composition leading to a greater explosive power, a less likelihood that the TNT will melt out when stored at a high temperature or that the final cast will possess cracks.

The following examples will illustrate how effective the replacement may be.

TABLE II

| Composition                                                                                 | Control                              | A     | B     | C     | D     | Control |
|---------------------------------------------------------------------------------------------|--------------------------------------|-------|-------|-------|-------|---------|
| RDX                                                                                         | 0                                    | 18.4  | 36.8  | 55.2  | 73.6  | 60      |
| TNT                                                                                         | 100                                  | 73.6  | 55.2  | 36.8  | 18.4  | 40      |
| Prepolymer                                                                                  |                                      | 4     | 4     | 4     | 4     |         |
| Polyol Curing Agent                                                                         |                                      | 2     | 2     | 2     | 2     |         |
| Melt Compatibilizer                                                                         |                                      | 2     | 2     | 2     | 2     |         |
| Characterization                                                                            | Rate of detonator, meters per second | 6,640 | 6,800 | 7,300 | 7,600 | 7,900   |
| Cast density, g./cc.                                                                        |                                      | 1.56  | 1.60  | 1.63  | 1.65  | 1.67    |
| 200 g. Bomb Brisance, sand crushed, g.: Detonator chg. wt., 0.2 gm. azide, 0.1 gm. tetralin | 48.0                                 | 50    | 51    | 52    | 54.6  | 54.6    |
| 40 hr. Vacuum stability, 120° C., 5 gms., ml. gas                                           | 0.20                                 | 1.0   | 1.0   | 1.0   | 0.7   | 0.3     |
| Explosol temp., 5 sec. ° C. (to decomposition)                                              | 475                                  | 400   | 300   | 300   | 275   | 280     |
| Impact Sensitivity, 2 kg. wt. ht. in inches (.017 mg. in confined cup)                      | 14                                   | 17    | 17    | 17    | 17    | 14      |
| Hardness, Shore D                                                                           | 145                                  | 45    | 50    | 55    | 65    | 145     |
| Brittleness, falling ball, 1/2 lb. steel ball, approx. height to cause fracture, inches     | 2                                    | 8     | 8     | 8     | 8     | 2       |
| Remarks: Melt Pouring temp., ° C.                                                           | 85                                   | 85    | 85    | 85    | 85    | 85      |
| Curing temperature                                                                          | (2)                                  | (2)   | (3)   | (3)   | (3)   | (2)     |
| Physical properties                                                                         | (1)                                  | (1)   | (1)   | (1)   | (1)   | (1)     |
| Exuding in shell, 71° C.                                                                    | Yes                                  | None  | None  | None  | None  | Yes     |
| Temperature cycling, -40° C. to +71° C.                                                     | (9)                                  | (7)   | (7)   | (7)   | (7)   | (9)     |
| Suspension or Settling out of RDX or HMX filler in melt phase                               | (2)                                  | (8)   | (8)   | (8)   | (8)   | (9)     |
| Temperature of melting-out of TNT, ° C.                                                     | 80                                   | 90    | 95    | 105   | 105   | 80      |

<sup>1</sup> Brittle. <sup>2</sup> N/a. <sup>3</sup> Room temperature 71° C. <sup>4</sup> Non-brittle.

<sup>5</sup> No cracks. <sup>6</sup> Suspension. <sup>7</sup> Settling out.

5 tags with results similar to that obtained in Table II may be achieved, if the polyurethane modified TNT is replaced with up to 80% HMX.

Obviously, many modifications and variations are possible in light of the above teachings. It is therefore to be understood that within the scope of the appended claims, the invention may be practiced otherwise than as described.

I claim:

10 1. A composition of a high explosive cast which is free of voids, cavitations, and exudation of oils up to a temperature of 71° C. consisting of

(a) 55 to 95 percent by weight of 2,4,6-trinitrotoluene, and

15 (b) 5 to 45 percent by weight of the reaction product of 2,4-tolylene diisocyanate and 1,4-butylen oxide polyglycol.

20 2. The composition of claim 1 wherein cyclotrimethylene trinitramine is substituted for up to 80 percent of the base weight of TNT in said composition.

3. The composition of claim 1 wherein cyclotetramethylene tetranitramine is substituted for up to 80 percent of the base weight of TNT in said composition.

4. The composition of claim 1 wherein said reaction

5 <sup>8</sup> Elastomeric. <sup>6</sup> Cracks develop.

product is accompanied by a polyol curing agent selected from the group consisting of castor oil and hydrogenated castor oil.

50 5. The composition of claim 4 wherein said reaction product is accompanied by poly-methyl styrene.

#### References Cited

#### UNITED STATES PATENTS

|              |         |                 |          |
|--------------|---------|-----------------|----------|
| 55 3,049,454 | 8/1962  | Stark           | 149—92   |
| 3,141,294    | 7/1964  | Lawrence et al. | 149—19   |
| 3,238,245    | 3/1966  | Reedy           | 149—93 X |
| 3,309,247    | 3/1967  | Bluhn           | 149—19 X |
| 3,350,245    | 10/1967 | Dickinson       | 149—19   |

60 BENJAMIN R. PADGETT, Primary Examiner.

U.S. CL. X.R.

65 149—92, 93, 105